

## UNITED STATES PATENT OFFICE.

EMILE BRONNERT, OF MULHOUSE, FRANCE.

MANUFACTURE OF ARTIFICIAL SILK.

No Drawing.

Application filed August 25, 1921. Serial No. 495,945.

*To all whom it may concern:*

Be it known that I, EMILE BRONNERT, a citizen of the Republic of France, residing at Mulhouse, Alsace-Lorraine, France, have invented certain new and useful Improvements in the Manufacture of Artificial Silk; and I do hereby declare the following to be a full, clear, and exact description of the invention.

According to a suggestion made some time ago by the present applicant, very fine threads of viscose silk were produced by the fine-spinning process, which allows of very strong precipitants such as sulphuric acid being employed and of the spinning, from the same viscose, of threads of all finenesses by means of nozzle apertures possessing the same mean diameter (0.10 mm.), by reason of the concentration of the acid being regulated according to the known rule and the flow of the viscose being adjusted according to the thickness of the thread to be obtained.

In the manufacture from viscose silk of artificial silk of about 8 deniers, the method is also known of adding glucose and other organic substances to the acid so as to deprive the acid of its sharpness.

A precipitating bath for viscose threads has already been suggested, consisting of a crude mixture of carbo-hydrates, mineral acid or salts of mineral acid and by-products obtained by hydrolyzing and heating wood or other cellulose-containing materials with mineral acids, with or without the addition of other reagents.

The present invention does not relate to these known methods but assumes for its starting point the observed fact that the threads obtained by the new fine-spinning process with a highly concentrated acid, often do not possess the requisite degree of flexibility and that the fine threads emerging from the nozzle show a strong tendency to knot together in a bunch, which must afterwards be disentangled.

The present invention provides a remedy for this disadvantageous behaviour. It consists in utilizing, for the maintenance of the degree of acidity in the spinning bath, instead of pure acid, acid containing in solution hydrolyzed dextrinous substances as hydrolyzed starch or either cellulose or coagulated waste viscose; (the latter forming a troublesome waste product arising during the filtration and transport of viscose solu-

tions). These products, when dissolved without heating in an excess of sulphuric acid, give rise to dextrinous products which act in the beneficial manner described.

Example I.—In a warm spinning bath, containing 150 grammes of sulphuric acid and 370 grammes of sodium sulphate per litre, the usual operation of spinning is carried out with crude viscose of a maturity represented by 9 sal ammoniac degrees. Supple threads of a brilliant beauty are obtained.

The previous dissolving in the acid of a quantity of cellulose hydrate waste represented by 75 grammes net weight had no effect on the qualities of the threads obtained. The excess of neutral salt  $\text{Na}_2\text{SO}_4$  over the proportion of bisulphate was in itself, sufficient to obviate any injurious dissociation.

Example II.—In a warm spinning bath, containing 250 grammes of sulphuric acid and only 250 grammes of soda per litre, the same viscose (9 degrees) is spun in the same way. The threads now obtained possess only a feeble brilliancy. If however part of the sulphuric acid be present in the bath in the form of a compound cellulose sulphur acid containing for instance a net weight of 80 grammes cellulose, then a thread of brilliant beauty is obtained. The astonishing result of the partial combination of the acid with the complex organic radicle is thus clearly evidenced.

Example III.—If, in Example II, the viscose employed be very fresh, having a maturity of about 11.5°, the preliminary dissolving of 80 grammes of cellulose in the acid, in a cold and concentrated condition, and its subsequent dilution with enough water to make it up to one litre, is inadequate for the production of highly brilliant threads, it is necessary to dissolve 100 grammes of cellulose and even more.

I claim:

1. A process of manufacturing very fine threads from viscose, which comprises regulating the rate of flow of the viscose from the forming nozzle, regulating the concentration of the acid hardening bath in accordance with the thread diameter desired, by increasing the strength of the acid according to the fineness of the threads, the strength of said bath being maintained by an aqueous solution of a like acid containing decomposed viscose.

2. A process of manufacturing very fine threads from viscose which comprises regulating the rate of flow of the viscose from the forming nozzle and the concentration of 10  
5 the acid hardening bath in accordance with the thread diameter desired, and maintaining the strength of said bath by an aqueous solution of a like acid containing viscose

that had been previously decomposed into cellulose hydrate.

In testimony that I claim the foregoing as my invention I have signed my name.

DR. EMILE BRONNERT.

Witnesses:

AMÉLIE BRONNERT,  
RENÉE BRONNERT.